

Patented Aug. 8, 1933

1,921,780

# UNITED STATES PATENT OFFICE

1,921,780

## WOOD FIBER MASS

Fritz Rühlemann, Wolfsgrun, and Otto Rudolf Herdey, Bautzen, Germany

No Drawing. Application August 15, 1931, Serial No. 557,426, and in Germany September 11, 1930

5 Claims. (Cl. 92—3)

The present invention relates to a new product made from wood, being in the form of a loose mass of wood fibers substantially individually free and readily reconverted into pulp by mechanical means or by being immersed in liquids.

One of the objects of the invention is to produce a loose mass of wood fiber, or mechanical wood pulp, from which the cementing-agents and adhesive substances have been removed to a greater or lesser extent.

A further object of the invention is to produce mechanical wood pulp of such a nature as will readily lend itself to further disintegration and manufacture into commercial products.

Other objects of the invention will become apparent from the further description hereinbelow and the claims.

Wood or wood-like plants, mechanically disintegrated by means of grinding stones or in any other manner into fibers and fiber bundles, are termed groundwood or mechanical wood pulp.

Originally the groundwood, after partial removal of the water, was filled into sacks and sold in a wet condition. Later on, the removal of the water was more thoroughly carried out on drying machines or in presses, and the groundwood was sold commercially in the form of moist or dry sheets, rolls, lumps or in loose form. Besides the individual fibers and fiber bundles, groundwood is chiefly composed of fiber fragments and fiber mucilage. During the extraction of the water, and in greater measure during the drying operation, the fiber fragments and fiber mucilage produce a cementitious substance which joins the fibers firmly together. By placing the groundwood upon a sieve or a paper machine wire, either in thin or thick layers, for the extraction of the water, paper or cardboard is produced.

The effect of pressure during the extraction of water and the drying operation while the groundwood is being formed into cardboard, etc., causes the fiber structure to be firmly and intimately interfelted. The cementing together of the individual fibers with each other is thereby considerably increased, so that the subsequent disintegration of the dried groundwood into dried fibers is possible only with special machines requiring considerable power and causing the fibers to lose their original character. Groundwood of this nature is suitable only for the manufacture of paper, board and cardboard, for which the cementing together of the individual fibers with the fiber fragments and fiber mucilage is a nec-

essary condition. Consequently the uses for groundwood of this description are limited.

The cementing together of the individual fibers through the fiber fragments and fiber mucilage also occurs when a fibrous felt is being formed from groundwood by means of suction—i. e., without presses—and by drying in a vacuum. It is therefore not possible again to disintegrate groundwood from which the water has been removed and which has been dried in this manner, into its original loose fibers without injuring them.

In order to find added uses for wood after it has been reduced mechanically into individual fibers and fiber bundles, it is important, according to the invention, to remove the causes which produce the cementing together of the individual fibers.

The invention relates to the production of a mass of wood fibers which consists exclusively of long individual wood fibers and fiber bundles and is completely free from fiber mucilage and poor in fiber fragments.

In order more easily to attain this object, the percentage of fiber fragments and fiber mucilage, in comparison with the long fibers, can be kept correspondingly small even during the original mechanical disintegration of the wood. It is important that the fiber mucilage and the colloidally dissolved fiber fragments be completely removed by washing. This makes it possible again subsequently to disintegrate the dried material into the form of uninjured original fibers. While, however, the disintegration of the wood into the commercially known groundwood or mechanical wood pulp, in which a large percentage of short fibers and especially of fiber fragments and fiber mucilage is desirable, is possible by the expenditure of a great deal of power, the new above mentioned method of the disintegration of the wood into long fibers and fiber bundles requires a considerably smaller amount of power.

The new wood fiber mass has a loose, homogeneous fibrous structure which is not cemented together nor interfelted and which resembles the structure of raw cotton.

The new wood fiber mass is ordinarily and commercially sold airdry in the form of thick sheets or cakes or in other desired form. The separation of the fibers of this wood fiber mass for conversion can be effected with the least consumption of power in a dry condition by known means, as for instance by carding and the like. The dry wood fiber mass, reduced to individual fibers, can be used for example when the

product to be made from it does not permit the addition of water, so that a blending of the wood fibers with pulverized substances or an impregnation of the wood fibers with water-repelling liquids can be undertaken.

For uses which require the addition of water the dried wood fiber mass can be reduced to its individual, uninjured original fibers simply by soaking the mass in a liquid. The wood fiber mass can also be converted directly from a pulpy condition, that is to say, prior to the removal of the water and the drying of the same. A special advantage of the new wood fiber mass consists in the fact that the disintegration of the wood fiber mass, from which the water has been extracted without pressure, is accomplished more easily and with considerably less consumption of power than is the case with the groundwood above mentioned, namely that from which the water has been removed by means of pressure.

The new wood fiber mass can be produced, for instance, in the following manner:

The wood or wood-like plants are mechanically disintegrated with the addition of water by means of the usual wood grinders or wood chopping machines in combination with rasps, mills, etc., wherein it is of advantage to be careful to preserve the long fibers and fiber bundles. The fiber pulp thus obtained is subjected to a washing operation with water which completely removes the fiber-mucilage and the colloidally dissolved fiber fragments from the mass. After the removal of these substances, the mass is ready for conversion into articles by processes in which the presence of water is required or not deleterious. If, on the other hand, the wood fiber mass is required to be dry for further conversion, the water is removed and the material dried, for example in rotating perforated drums through which air flows, but without special application of pressure. Other known equipment may also be used for the removal of the water and for the drying, such as cylinder-and flat wire wet machines, vacuum installations or drains, drying cylinders and the like. The main object is to avoid the use of undue pressure which would result in undesired felting of the fibers.

50

125

55

130

60

135

65

140

70

145

75

150

The described properties of the new wood fiber mass offer chiefly the possibility to use the same for the manufacture of certain synthetic material, for litter, for a material for absorbing liquids, and for the production of heat-, cold- and sound-insulating substances. Moreover it has now only become possible through the use of this new dry wood fiber mass to produce mixtures thereof with pulverized binding materials which on addition of water, and after swelling, take on solid forms.

The wood fiber mass described is an entirely new product which can be used either by itself or as primary material for conversion into other products.

We claim:

1. The process of producing a loose mass of groundwood fibers which comprises grinding wood in presence of water to produce individual fibers and fiber bundles, washing fiber-mucilage and colloidally dispersed fibers from the resulting mass, and drying the latter without application of substantial pressure.

2. The process of producing wood fiber free from slimy particles and water-soluble matter which comprises grinding wood in the presence of water to produce individual fibers and fiber-bundles, and washing said fibers and fiber-bundles substantially free from said particles and soluble matter.

3. The process of producing wood fiber free from slimy particles and water-soluble matter which comprises comminuting wood to produce loosened woody fibers and fiber-bundles and washing the same with water to remove therefrom slimy particles and water-soluble gums.

4. As a new product, a mechanically disintegrated wood fiber mass from which water-soluble matter and slimy particles have been removed by washing merely with water.

5. As a new product, a mechanically disintegrated wood fiber mass from which water-soluble matter and slimy particles have been removed by washing merely with water and which has been dried without application of pressure.

FRITZ RÜHLEMANN.

OTTO RUDOLF HERDEY.

120

110